

## UNITED STATES PATENT OFFICE

EDWARD TOMAN, OF CHICAGO, ILLINOIS, ASSIGNOR TO E. TOMAN & COMPANY, OF CHICAGO, ILLINOIS, A CORPORATION OF ILLINOIS

## METHOD OF MAKING MOLDS

No Drawing.

Application filed July 6, 1931. Serial No. 549,097.

This invention relates to a method of forming molds, particularly such as are used in the making of the castings of non-ferrous metals.

5 In the making of molds of such materials as calcium sulphate, or plaster of Paris, which depend upon water of crystallization for their set, it has been the custom to mix the sulphate and water together in a separate

10 puddling operation to form a plastic material. The plastic is then forced into a flask and about a pattern or form. A wire brush or similar instrument is used in order to pack the material about the form, and also to penetrate any air bubbles which might form in the material. The purpose is to secure a uniform and dense deposit of the plastic about the form.

Such a method has the disadvantage that 20 the plaster of Paris reacts with the water so rapidly that the water is largely used up and the material partially set before it can be properly packed into the mold. Therefore it is extremely difficult, even with utmost care, 25 to secure uniformity by puddling the plastic separately and then applying it to a mold with the use of a brush.

It is an object of this invention to provide a method of making molds which does 30 not have the above named disadvantages.

It is a further object of this invention to produce a mold by a method in which the hydrated form of the material is formed directly in the flask containing the pattern and 35 a rapid set is obtained.

It is a still further object of this invention to produce a mold by a method which insures that the maximum amount of water will be quickly taken up by the sulphate and that 40 the plastic mass will be uniform throughout.

These and further objects of this invention will be apparent from the following description of a preferred form and from the appended claims.

45 In carrying out this invention, a container, or flask, is provided, on the bottom of which the pattern or object is formed. The container preferably has easily assembled sides and end walls or barriers and a removable

50 cover.

Dry, finely powdered calcium sulphate, hemi-hydrate, or plaster of Paris, is placed in the flask above the pattern. The amount of plaster of Paris to be used is determined by the thickness desired to be given to the molds 55 and the pattern should be well covered throughout its extent by the powdered material. A predetermined amount of water is then added.

The sidewalls or barriers of the container 60 should be so proportioned to the pattern formed on the bottom that the water will be sufficiently high to permit a space for the hydrating action. A plate or cover is placed over the top of the barriers and the container 65 and contents is subjected to a rapid shaking.

The container is moved rapidly back and forth and up and down, and in fact in every direction at a high rate of speed, to distribute the water through the material. Such an action insures that the water will be distributed through the material in an even manner. The water is thus caused to travel at a high rate of speed through the plastic forming material and then to impact against the pattern 75 and cover plate. The surface tension is thus overcome, permitting the compacting of the plastic material at the very surface of the pattern. This thorough mixing of the water and material with the overcoming of the 80 surface tension of the water, guarantees that the minutest particles come in contact with the water.

As the water is mixed with the material, the latter begins to hydrate and gradually 85 set. The motion insures that there will be no air pockets formed, and also that the plastic material thus formed will be even throughout, and will closely follow the pattern or object.

90 The amount of water to be used is calculated from the following equation:



The molar proportion of plaster of Paris 95 to water is 1 to 3, or three parts by weight of water to sixteen parts by weight of plaster of Paris. The amount of water actually used is usually from 15 to 25 per cent in excess of the calculated amount.

It will be seen by this method, that the water comes into intimate contact with the minutest particles of the dried material, whereby very rapid and very thorough hydration is achieved. The mechanical motions of the particles and the water insure that not only will there be no air pockets but also the hydrated or plastic material thus formed will shape itself uniformly about the pattern.

Many changes may be made in the details and arrangements in carrying out the process and I do not wish to be limited otherwise than is necessary, by the prior art and the scope of the appended claims.

I am aware that numerous details of the process may be varied through a wide range without departing from the principles of this invention, and I, therefore, do not purpose limiting the patent granted hereon otherwise than necessitated by the prior art.

I claim as my invention:

1. The method of forming a mold, which comprises, adding a plaster forming powder to a container having a pattern formed on one wall thereof, the amount of the powder being sufficient to thoroughly cover the pattern, adding a predetermined amount of water, closing the container, vigorously agitating the container and contents to cause the contents to impact against the sides and top of the container to thereby cause the powder to thoroughly absorb the water and allowing the plastic mixture to set.

2. The method of forming a mold, which comprises adding powdered plaster of Paris to a flask having a pattern formed on one wall thereof, the amount of powder being sufficient to thoroughly cover the pattern, adding slightly more than enough water to change the powdered plaster of Paris to the hydrated form, closing the flask, vigorously agitating the flask and contents successively vertically and horizontally to cause the contents to impact against the side and top of the flask to thereby cause the powder to thoroughly absorb the water and allowing the hydrated form to set.

3. The method of forming a mold which comprises adding powdered plaster of Paris to a flask having a pattern formed on one wall thereof, in sufficient quantity to cover the pattern, adding slightly more than enough water to change the powdered plaster of Paris to the hydrated form, closing the flask and vigorously agitating the flask and contents to impact the contents against the pattern and the side and top of the flask to cause the powder to thoroughly absorb the water, and allowing the hydrated form to set.

In testimony whereof I have hereunto subscribed my name at Chicago, Cook county, Illinois.

EDWARD TOMAN.